

# UNITED STATES PATENT OFFICE.

ADOLF HERBIG, OF COLOGNE-BICKENDORF, GERMANY.

## VARNISH FOR PRODUCING MAT SURFACES.

No. 861,847.

Specification of Letters Patent.

Patented July 30, 1907.

Application filed April 3, 1906. Serial No. 309,725.

To all whom it may concern:

Be it known that I, ADOLF HERBIG, a subject of the German Emperor, and a resident of Cologne-Bickendorf, in the Kingdom of Prussia, German Empire, and whose post-office address is 210 Rochusstrasse, same place, have invented new and useful Improvements in Varnishes for Producing Mat Surfaces and in Processes for Making Same, of which the following is a full, clear, and exact specification.

10 Varnishes hitherto used for producing coatings having a mat surface consist either of wax, ceresin, ozokerite, paraffin or other solid hydrocarbon suspended in a fatty oil varnish or of a mechanical mixture of a fatty oil varnish with an indifferent material, like starch, 15 fine sand, certain silicates, gypsum or other inorganic so-called filling materials. These two kinds of mat varnishes leave much to be desired in that they produce very imperfect results in practice. In the first kind the wax, ceresin or other hydrocarbon takes no 20 part in the peculiar drying and consequent hardening process, because of its slight chemical activity, and there is also the objection that during the progressive drying of the oil varnish the tendency for the latter to dissolve the added matter decreases, so that this matter 25 accumulates on the surface of the coating, which thus acquires the property of becoming sticky and soft at temperatures whereat the added matter begins to become soft and fluid. On this account mat varnishes of this kind cannot be used for ordinary furniture, if 30 a good result is to be obtained. The varnishes of the second kind, so far as those containing starch or starchy materials are concerned, have the disadvantage that they cannot withstand contact with water without the swelling of the starch. Spots ensue and owing to the 35 unequal expansion of the swollen starch and oil varnish the whole coating cracks and peels off. The varnishes made with indifferent filling materials have the like disadvantage, that the filling material and the oil varnish surrounding it have an essentially different 40 tendency to take up moisture from the air; on this account coatings of such varnishes soon crack and become brittle so that they are not applicable, especially to large surfaces like cabinets or doors.

The present invention depends on the discovery that 45 when a fatty drying oil or a fatty drying oil varnish is mixed mechanically with hydrated alumina, the varnish and aluminum compound combine under partial saponification. But it is during the drying of the oil or varnish that chemical combination especially 50 occurs between it and the aluminum compound, as the acid compounds produced in the varnish by oxidation during the drying have a greater activity than that of the original oil or varnish and themselves combine with the basic aluminum compound. Evidence of the

correctness of the foregoing statements accrues from 55 the facts that already during the mechanical mixing of the aluminum compound with the fatty oil varnish, heat is evolved, indicating chemical reaction, and that the mixture undergoes a considerable change of consistency after a short time, showing that a new compound is being formed. The dried coating of the new compound displays its difference from the oil varnish containing indifferent filling materials by yielding the aluminum compound in a state of combination when treated with solvents. Under "fatty drying oils" 60 are understood vegetable oils which contain glycerids of unsaturated fatty acids and which are capable, when exposed to the oxygen of the air, of forming a tenacious skin within a shorter or longer period of time. Under "fatty drying oil varnishes" are understood 65 such vegetable oils that are boiled with or without addition of a gum or siccative in a suitable form and which are glycerids of unsaturated acids and which possess the property, when exposed to the oxygen of the air, to form a firm tenacious skin. This definition 70 corresponds to the definition given by Lewkowitsch in his standard work.

The mat varnish made according to the invention, unlike the aforesaid mat varnishes of the first kind, does not become sticky or show any tendency to soften; 80 as compared with mat varnishes of the second kind, it possesses complete homogeneity, whereby it remains elastic and free from cracks; moreover, the aluminum compound formed not being saponifiable, the varnish is not attacked by water at ordinary temperature. 85

Example. 90 parts of a fatty drying oil varnish are ground in known manner with 4-10 parts of hydrated alumina, and the strongly thickened product is reduced to the original consistence by addition of a suitable solvent. Such solvents are spirits of turpentine, 90 wood alcohol, the light distillation products of petroleum and coal-tar, acetone and its homologues, carbon tetrachlorid, carbon sulfid, amyl and other alcohols, acetic esters, nitrobenzene, anilin, and the like. The varnish thus prepared is ready for use. 95

What I claim is:—

1. The herein described varnish for producing mat surfaces, consisting of a mixture of a fatty drying oil with hydrated alumina.

2. The herein described varnish for producing mat surfaces, consisting of mixture of a fatty drying oil varnish with hydrated alumina. 100

In testimony, that I claim the foregoing as my invention, I have signed my name in presence of two subscribing witnesses.

ADOLF HERBIG.

Witnesses:  
BESSIE F. DUNLAP,  
LOUIS VANDORN.